

## UNITED STATES PATENT OFFICE

CAMILLE DREYFUS, OF NEW YORK, N. Y., AND GEORGE RIVAT, OF PATERSON, NEW JERSEY, ASSIGNORS TO CELANESE CORPORATION OF AMERICA, A CORPORATION OF DELAWARE

## DIFFERENTIALLY COLORING FABRIC AND PRODUCT THEREOF

No Drawing. Application filed April 13, 1929. Serial No. 354,982.

This invention relates to a differentially colored fabric and process of producing the same by treating fabrics in conjunction with either resist printing or discharge printing with a dyestuff of the aniline black type.

An object of our invention is to produce prints having dark backgrounds and light colored designs on fabrics and particularly fabrics containing organic derivatives of cellulose such as cellulose acetate.

A further object of our invention is to produce resist or discharge prints using a dye-stuff of the steam aniline black type. Other objects of our invention will appear from the following detailed description.

The production of prints having dark backgrounds and light colored designs on fabrics containing organic derivatives of cellulose, such as cellulose acetate, has presented serious problems. This is due to the fact that the dyestuffs that impart a dark color to this fabric cannot be readily discharged by the ordinary discharge pastes used in the printing art. We have found, however, that if pastes containing an alkali and a reducing agent are applied to a fabric prior to its being treated with the aniline black base, as in resist printing, or after the application of the aniline black base, but prior to steaming or otherwise oxidizing after the discharge printing, light colored designs on dark backgrounds may be produced.

In accordance with our invention we produce light colored designs on dark backgrounds by resist or discharge printing fabrics containing organic esters of cellulose by treating the same with a paste containing alkali or reducing agent or both, with or without coloring matter. In our process the fabric is padded with a material containing steam aniline black paste, either before or after the application of the paste containing the alkali and/or reducing agents.

The fabric to be treated in accordance with our invention may contain yarns made of any organic derivatives of cellulose and particularly organic esters of cellulose such as cellulose acetate, cellulose formate, cellulose propionate and cellulose butyrate, or cel-

lulose ethers such as ethyl cellulose. The fabric need not necessarily consist wholly of yarns made of these organic derivatives of cellulose but may also contain yarns of other fibres such as cotton, silk, or reconstituted cellulose (rayon). Examples of such mixed fabric are mixed cellulose acetate and silk and mixed cellulose acetate and cotton.

The paste to be used for the resist or discharge printing as stated before contains both alkali and reducing agent. The alkali used may be sodium hydroxide or potassium hydroxide or alkaline salts such as sodium carbonate.

Of the reducing agents that are suitable, we have found that although the sodium, zinc or potassium hydrosulphites give satisfactory results, lykopon and protoline (zinc formaldehyde sulphoxylate) give superior results. The action of the reducing agent is to prevent the oxidation of the aniline black base to a dark colored body on subsequent steaming. As stated before, the paste contains alkali and reducing agent. If colored discharge prints are desired, the paste may contain vat colors, SRA dyes or any direct dyes for the cellulose acetate fabrics.

The paste containing the dye of the aniline black type contains preferably aniline hydrochloride, ferrocyanide and also acids, catalysts, oxidation agents and thickening agents. The aniline black material is preferably a combination known as Steam Aniline black which may be prepared by mixing ferrocyanide, potassium chlorate, aniline chloride, water, glacial acetic acid, glycerine and gum tragacanth.

Of the acids that are to be used, we prefer the aliphatic acids such as acetic acid. Examples of catalysts or oxygen carriers appropriate for use in the paste are cupric chloride or copper sulphate or mixtures of these. Examples of oxidizing agents are sodium chloride or potassium chloride. Any suitable thickening material, such as gum tragacanth, gum arabic or British gum may be used.

If resist printing is desired, the paste containing alkali and reducing agent is applied before padding with the aniline oil material. After the aniline oil black material is applied,

the fabric is steamed in order to oxidize the same to a black color. However, at those places where the resist paste has been applied, no oxidation of the aniline black base takes 5 place.

If discharge printing is to be effected, the aniline black paste is applied first, and then the fabric is printed with the paste containing the alkali and reducing agent, after which 10 the fabric is steamed to oxidize the aniline black that is on the unprinted portion of the fabric. Care should be taken that the fabric having the aniline black base thereon is not steamed before the discharge paste is applied, 15 since once the black color is developed by steaming it does not readily discharge.

In order to prevent halo effects which may occur by the use of the methods disclosed in this application, it is well to pad the fabric 20 with aluminum acetate or sodium acetate prior to applying the printing paste containing the alkali and reducing agent, either before or after application of the paste containing the aniline black base. Or else, the 25 sodium acetate or aluminum acetate may be added to the resist or discharge paste containing the alkali and reducing agent.

The goods to be treated in accordance with this invention may or may not be subjected 30 to an iron proofing treatment before being processed. The goods are printed dry after first being properly stripped down. Where white discharges or prints on black backgrounds are desired, it is advisable to add 35 some zinc oxide to the paste to act as a pigment, resulting in a clear bright white.

It has also been found that the addition of alcohol to the resist paste results in a better penetration of the paste throughout the 40 cellulose acetate fabrics. Other swelling agents such as the glycol derivatives, pyridine, triethylamine and the like can also be employed. We have also found that the presence of aluminum or chromium chloride 45 in the paste can be advantageously dispensed with where bright white discharges are desired. This is very probably due to the fact that some oxidation of the aniline takes place immediately upon contact with these substances even before steaming.

As stated before, the paste containing the alkali and reducing agent prevents the oxidation, during steaming, of the aniline black on that part of the fabric to which it has been 55 applied.

The goods are steamed after the paste containing the alkali and/or reducing agent has been applied, and after they have been padded with a paste containing the aniline black base. This causes the aniline black base to 60 become oxidized on that part of the fabric that does not have the paste containing alkali and reducing agent applied thereto, thus producing light colored figures on black backgrounds.

The paste containing alkali and reducing agent may be applied by suitable engraved or embossed rolls, plates or blocks. It also may be applied by brushing or spraying through stencils having desired designs. 70

In order to further illustrate our invention, specific details will now be given with respect to the use of an aniline black base, in order to obtain a white resist on a black background. 75

#### Example

This example is for resist printing, that is where the paste is applied to the fabric before the aniline paste is applied thereto. 80

After the fabric has been properly stripped down, with or without iron proof treatment, and dried, it is printed, in any desired pattern, with the following paste:

|                          | Parts     | 85 |
|--------------------------|-----------|----|
| Zinc oxide               | 100       |    |
| Protoline                | 100       |    |
| Sodium oxalate           | 100       |    |
| Caustic soda             | 50 to 100 |    |
| Water                    | 350       | 90 |
| Gum tragacanth (60/1000) | 400       |    |
| Alcohol (by weight)      | 40        |    |

The fabric after being printed with the above paste is dried at 60° C. and then padded by a millepoint roller, with steam aniline black paste. This paste is obtained by mixing together the three following solutions immediately before using. 85

|                        | Parts | 100 |
|------------------------|-------|-----|
| Potassium ferrocyanide | 100   |     |
| Potassium chlorate     | 160   |     |
| Water                  | 1000  |     |

|                       | Parts | 165 |
|-----------------------|-------|-----|
| Aniline chloride      | 420   |     |
| Water                 | 400   |     |
| Acetic acid (glacial) | 1000  |     |
| Glycerine             | 80    | 110 |

|                          | Parts |  |
|--------------------------|-------|--|
| Gum tragacanth (60/1000) | 1000  |  |

The fabric after having been printed with the steam aniline black paste is steamed in the Mather Platt steamer from 5 to 10 minutes. It is then washed out in water at 50° C. and then chromated with 4% of bichromate and 4% of an aniline chloride solution prepared by mixing together 1430 grams of aniline chloride and 3 litres of water. (The percentages above given are figured on the weight of the fabric being treated.) After the chromating treatment above outlined, the fabric is washed out slightly, soaped at 50 to 60° C. and rinsed well. 115

The fabric after the above treatment will be found to have a bright white pattern upon a deep black background. The pattern will 120 125 130

- be clear cut and distinct with no semblance of halos present.
- Due to the composition of the paste employed, no oxidation of the aniline takes place until the steaming treatment is applied. This prevents the slight darkening of the resist portions which occurs in processes heretofore employed and results in a bright white print on a black background. Where it is desired 1) to increase the speed of the oxidation, the same may be effected by adding one gram of copper sulphate in 100 cc. of water to the paste, although such addition is not necessary.
- 15 It is to be understood that the foregoing detailed description is given merely by way of illustration and that many variations may be made in the compositions employed and the procedure followed without departing 20 from the spirit of the invention. The process and compositions above outlined can be employed for discharge printing as well as for resist printing.
- Having described our invention, what we 25 claim and desire to secure by Letters Patent is:
1. Method of producing differential colored effects on fabrics containing organic derivatives of cellulose which comprises applying 30 locally to said fabric a paste comprising a reducing agent, an alkali, a swelling agent for the cellulose derivative and a pigment and subsequently treating the fabric with a paste containing an aniline black base and an oxidizing agent and then steaming the fabric.
2. Method of producing differential colored effects on fabrics containing organic derivatives of cellulose which comprises applying 35 locally to said fabric a paste comprising a reducing agent, an alkali, a swelling agent for the cellulose derivative and a pigment and subsequently treating the fabric with a paste containing an aniline black base, a ferrocyanide and an oxidizing agent and then 40 steaming the fabric.
3. Method of producing differential colored effects on fabrics containing organic derivatives of cellulose which comprises applying 45 locally to said fabric a paste containing protoline, caustic soda, zinc oxide and alcohol, and subsequently treating the fabric with a paste containing an aniline black base and an oxidizing agent and then steaming the fabric.
4. Method of producing differential colored 50 effects on fabrics containing organic derivatives of cellulose which comprises applying locally to said fabric a paste containing protoline, caustic soda, zinc oxide and alcohol, and subsequently treating the fabric with a 55 paste containing an aniline black base, an oxidizing agent, a ferrocyanide and acetic acid and then steaming the fabric.
5. Method of producing differential colored 60 effects on fabrics containing cellulose acetate which comprises applying locally to
- said fabric a paste containing protoline, caustic soda, zinc oxide and alcohol, and then steaming the fabric, and subsequently washing the same with warm water and treating the washed fabric with a solution containing 70 a bichromate and aniline chloride.
6. Method of producing differential colored effects on fabrics containing cellulose acetate which comprises applying locally to 75 said fabric a paste containing protoline, caustic soda, zinc oxide and alcohol, and then steaming the fabric, and subsequently washing the same with warm water and treating the washed fabric with a solution containing a bichromate and aniline chloride.
- In testimony whereof, we have hereunto subscribed our names.
- CAMILLE DREYFUS.  
GEORGE RIVAT.
- 80  
85  
90  
95  
100  
105  
110  
115  
120  
125  
130